



US008741532B2

(12) **United States Patent**  
**Zhou et al.**

(10) **Patent No.:** **US 8,741,532 B2**  
(45) **Date of Patent:** **Jun. 3, 2014**

(54) **TONER WITH IMPROVED CHARGING**

(75) Inventors: **Ke Zhou**, Oakville (CA); **Shigang Qiu**,  
Toronto (CA); **Kimberly Nosella**,  
Mississauga (CA); **Cuong Vong**,  
Hamilton (CA)

(73) Assignee: **Xerox Corporation**, Norwalk, CT (US)

(\*) Notice: Subject to any disclaimer, the term of this  
patent is extended or adjusted under 35  
U.S.C. 154(b) by 0 days.

(21) Appl. No.: **13/251,161**

(22) Filed: **Sep. 30, 2011**

(65) **Prior Publication Data**

US 2013/0084519 A1 Apr. 4, 2013

(51) **Int. Cl.**  
**G03G 5/00** (2006.01)

(52) **U.S. Cl.**  
USPC ..... **430/137.14; 430/109.1**

(58) **Field of Classification Search**

USPC ..... 430/108.1, 109.1, 109.4, 137.14  
See application file for complete search history.

(56) **References Cited**

U.S. PATENT DOCUMENTS

|                   |        |                        |           |
|-------------------|--------|------------------------|-----------|
| 2006/0051581 A1 * | 3/2006 | Yamamoto et al. ....   | 428/402   |
| 2007/0207397 A1 * | 9/2007 | Julien .....           | 430/107.1 |
| 2008/0107989 A1 * | 5/2008 | Sacripante et al. .... | 430/109.4 |
| 2009/0180807 A1 * | 7/2009 | Mitsumori et al. ....  | 399/220   |
| 2010/0248112 A1 * | 9/2010 | Fukushima et al. ....  | 430/105   |

\* cited by examiner

*Primary Examiner* — Stewart Fraser

(74) *Attorney, Agent, or Firm* — MDIP LLC

(57) **ABSTRACT**

The disclosure describes a toner process in which portion-wise addition of colorant(s) during particle formation is used to control the distribution of colorant within the toner particle, thereby enhancing A zone charge.

**20 Claims, No Drawings**

## 1

## TONER WITH IMPROVED CHARGING

## FIELD

Toners made by adding colorant in plural separate portions, which show improved A zone charging for use in developers; developers comprising said toner; devices comprising said toner and developers; imaging device components comprising said toner and developers; imaging devices comprising said toner and developers; and so on, are described.

## BACKGROUND

Carbon black is a commonly used black colorant of high color density (coloring per unit weight), a high blackness degree and high light fastness. In efforts to increase toner pigment loading using carbon black, it was revealed that such hyperpigmented black toners exhibited lower charging with high dielectric loss, both of which reduce transfer efficiency and degrade image quality. Black pigments are known to be more conductive than other pigments, however, such carbon black pigments form conductive pathways through the toner particle resulting in the defects or limitations discussed above.

Therefore, there remains a need to increase pigment loading without adversely impacting toner properties, for example, by maintaining or enhancing charging to enable lower cost hyperpigmented toners, black toners and so on.

## SUMMARY

The instant disclosure describes a toner process in which portion-wise addition of a colorant is used to control the distribution of colorant within the toner particle. By adding colorant, for example, in two portions, in a toner emulsion/aggregation process, toner charge and operability, for example, under high humidity conditions are improved, perhaps by minimizing the formation of conductive pathways through the toner.

In embodiments, a method for making a toner is disclosed including combining an amorphous resin, such as, a low molecular weight (LMW) amorphous resin, a high molecular weight (HMW) amorphous resin or both, an optional crystalline resin, an optional wax, a first colorant, and optionally, a second colorant to form a mixture; adding a flocculent to the mixture to form a particle; adding a third colorant and optionally, a fourth colorant to form a core particle; aggregating the core particle to a larger size; optionally adding a shell resin to form a core-shell particle; quenching and coalescing the core particle or core-shell particle; and obtaining the core particles or core-shell particles to form a toner, where the resulting toner exhibits higher charging and improved performance, for example, under high humidity, as compared to the same toner prepared by adding the first and third colorants at the same time before the first particle is obtained. In embodiments, the first and third colorants are the same color. In embodiments, the second and fourth colorants are the same color. In embodiments, the first and third colorants are the same pigment. In embodiments, the second and fourth colorants are the same pigment. In embodiments, colorants are added at additional time points, wherein colorants can be the same or different. In embodiments, colorants are added continuously or are metered into a reaction mixture.

In embodiments, the first colorant is a black. In embodiments, a second colorant is used. In embodiments, the second colorant is a cyan. In embodiments, the third colorant is a black. In embodiments where the colorants are the same, the

## 2

colorant is introduced in portions during particle development. The colorant can be introduced in two or more portions as a design choice. The colorant can be added continuously.

In embodiments, a method for making a black toner is disclosed including combining an amorphous resin, such as, an LMW amorphous resin, a HMW amorphous resin or both, an optional crystalline resin, an optional wax, a black colorant, and an optional first colorant to form a mixture, adding a flocculent to said mixture to enable aggregation of particles; 5 adding further black colorant and optionally, a second colorant and enabling further aggregation to form larger particles; optionally adding a shell resin to form core-shell particles; quenching and coalescing the particles or core-shell particles; and obtaining the particles or core-shell particles to comprise 10 a black toner. In embodiments, the black colorant and the further black colorant are the same. In embodiments, the first colorant and the second colorant are the same. In embodiments, the first colorant, the second colorant or both are a cyan. In embodiments, the amount of the further black colorant added to the composition after said particles are formed is greater than the amount of the black colorant added before the particles are formed from the initial mixture. In embodiments, the amounts of all colorants are the same. In embodiments, the black colorant and the further black colorant are 15 the same black pigment. In embodiments, the black pigment comprises a furnace black and exhibits one or more of the following properties: a BET surface area of about 65 m<sup>2</sup>/g; an oil absorption number (OAN) of about 42 ml/100 g; or about 20 0.5% volatile matter at 950° C.

30

## DETAILED DESCRIPTION

## I. Carbon Black

Carbon black is virtually pure elemental carbon in the form of particles produced by incomplete combustion or thermal decomposition of gaseous or liquid hydrocarbons. The physical appearance is that of a black, finely divided pellet or powder. The particles can have a specific surface area, particle size, structure, conductivity and color, as known in the art.

35 The conductivity of carbon black is dependent on a number of properties including surface area and structure. Generally, the greater the surface area and the greater the structure, the more conductive the carbon black. Surface area can be measured by the BET (Brunauer Emmett Teller) method, and the nitrogen absorption surface area per unit weight of carbon black is a measure of primary particle size. Structure is a complex property that relates to the morphology of the primary aggregates of carbon black. Structure is a measure of both the number of primary particles comprising a primary aggregate and the manner in which the particles are fused together. High structure carbon blacks are characterized by aggregates comprised of many primary particles with considerable branching and chaining, while low structure carbon blacks are characterized by compact aggregates comprised of 40 50 a few primary particles.

55 Carbon black frequently is identified by designating the method of preparation, e.g., channel black, lampblack, furnace black, oil black and thermal black. In embodiments, a carbon black useful in the present disclosure may be furnace black, e.g., but not limited to, NIPex® 35. NIPex® 35 is a furnace black with an average primary particle size of about 31 nm and a BET surface area of about 65 m<sup>2</sup>/g. NIPex® 35 may exhibit a neutral to blue undertone and is sold worldwide.

60 Unless otherwise indicated, all numbers expressing quantities and conditions, and so forth used in the specification and claims are to be understood as being modified in all instances by the term, "about." "About," is meant to indicate a variation

of no more than 20% from the stated value. Also used herein is the term, "equivalent," "similar," "essentially," "substantially," "approximating" and "matching," or grammatical variations thereof, have generally acceptable definitions or at the least, are understood to have the same meaning as, "about."

In the application, use of the singular includes the plural unless specifically stated otherwise. In the application, use of, "or," means, "and/or," unless stated otherwise. Furthermore, use of the term, "including," as well as other forms, such as, "includes," and, "included," is not limiting.

For the purposes of the instant disclosure, "toner," "toner composition," and "toner particles," can be used interchangeably, and any particular or specific use and meaning will be evident from the context of the sentence, paragraph and the like in which the word or phrase appears.

As used herein, "pH adjuster," means an acid, base or a buffer which may be used to change the pH of a composition (e.g., slurry, resin, aggregate, toner and the like). Such adjusters may include, but are not limited to, sodium hydroxide (NaOH), nitric acid, sodium acetate/acetic acid and the like.

As used herein, a, "colorant," generically encompasses pigments, dyes, which can be synthetic or naturally occurring, and so on, which can be a solid or a liquid, essentially an entity which imparts a color. Use of any one term for such a coloring agent, such as, a pigment or a dye, which terms are used herein interchangeably, includes the other forms as well. As used herein, any one particular colorant can be identified by a particular spectral color as commonly known, that is, for example, black, red, blue, cyan, yellow and so on. As used herein, use of a color, such as, black, is meant to encompass a black pigment, a black dye, a black colorant and so on, any other material that imparts a color.

As used herein, "hyperpigmented," means a toner having higher pigment loading at low toner mass per unit area (TMA) such as to provide a sufficient image reflection optical density of greater than 1.4 when printed and fused on a substrate, such pigment loading chosen so that the ratio of TMA measured for a single color layer in mg/cm<sup>2</sup> divided by the volume diameter of the toner particle in microns, is less than about 0.075 to meet that required image density.

## II. Toner Particles

Toner particles of interest comprise a resin, such as, an acrylate resin, a styrene resin, a polyester resin and so on, and thus, a resin-forming monomer(s) is reacted with suitable other reactants to form a polymer.

In embodiments, the resin comprises a polyester polymer, and in the context of a toner for use with certain imaging devices, comprises a polyester polymer that solidifies to form a particle. A composition can comprise more than one form or sort of polymer, such as, two or more different polymers, such as, two or more different polyester polymers composed of different monomers. The polymer can be an alternating copolymer, a block copolymer, a graft copolymer, a branched copolymer, a crosslinked copolymer and so on.

The toner particle can include other optional reagents, such as, a surfactant, a wax, a shell and so on. The toner composition optionally can comprise inert particles, which can serve as toner particle carriers, which can comprise a resin as taught herein. The inert particles can be modified, for example, to serve a particular function. Hence, the surface thereof can be derivatized or the particles can be manufactured for a desired purpose, for example, to carry a charge or to possess a magnetic field.

### A. Components

#### 1. Resin

Toner particles of the instant disclosure include a resin-forming monomer suitable for use in forming a particulate

containing or carrying a colorant of a toner for use in certain imaging devices. Examples include polyacrylates, polystyrenes, polyesters and so on as known in the art. The resin-forming monomer is one that is inducible to form a resin, that is, which reacts, sets or solidifies to form a solid. Such a resin, a plastic, an elastomer and so on, whether naturally occurring or synthetic, is one that can be used in an imaging device. In embodiments, any suitable monomer or monomers are induced to polymerize to form a polyester resin. Any polyfunctional monomer may be used depending on the particular polyester polymer desired in a toner particle. Hence, bifunctional reagents, trifunctional reagents and so on can be used. One or more reagents that comprise at least three functional groups can be incorporated into a polymer or into a branch to enable branching, further branching and/or crosslinking. Examples of such polyfunctional monomers include 1,2,4-benzene-tricarboxylic acid, 1,2,4-cyclohexanetricarboxylic acid, 2,5,7-naphthalenetetricarboxylic acid, 1,2,4-naphthalenetetricarboxylic acid, 1,2,5-hexanetricarboxylic acid, 1,3-dicarboxyl-2-methyl-2-methylenecarboxylpropane, tetra(methylene-carboxyl)methane and 1,2,7,8-octanetetracarboxylic acid.

One, two or more polymers may be used in forming a toner or toner particle. In embodiments where two or more polymers are used, the polymers may be in any suitable ratio (e.g., weight ratio) such as, for instance, with two different polymers, from about 1% (first polymer)/99% (second polymer) to about 99% (first polymer)/1% (second polymer), in embodiments from about 10% (first polymer)/90% (second polymer) to about 90% (first polymer)/10% (second polymer) and so on, as a design choice.

The polymer may be present in an amount of from about 65 to about 95% by weight, from about 70 to about 90%, from about 75 to about 85% by weight of toner particles on a solids basis.

#### a. Polyester Resins

Suitable polyester resins include, for example, those which are sulfonated, non-sulfonated, crystalline, amorphous, combinations thereof and the like. The polyester resins may be linear, branched, high molecular weight, low molecular weight, crosslinked, combinations thereof and the like. Polyester resins may include those described, for example, in U.S. Pat. Nos. 6,593,049; 6,830,860; 7,754,406; 7,781,138; 7,749,672; and 6,756,176, the disclosure of each of which hereby is incorporated by reference in entirety. Polyester resins, for example, can be used for applications requiring low melting temperature.

When a mixture is used, such as, amorphous and crystalline polyester resins, the ratio of crystalline polyester resin to amorphous polyester resin can be in the range from about 1:99 to about 30:70; from about 3:97 to about 25:75; in embodiments, from about 5:95 to about 15:95, or more crystalline polyester resin.

A polyester resin may be obtained synthetically, for example, in an esterification reaction involving a reagent comprising a carboxylic acid or an ester group and another reagent comprising an alcohol. In embodiments, the alcohol reagent comprises two or more hydroxyl groups, in embodiments, three or more hydroxyl groups. In embodiments, the acid comprises two or more carboxylic acid groups, in embodiments, three or more carboxylic acid groups. Reagents comprising three or more functional groups enable, promote or enable and promote polymer branching and crosslinking. In embodiments, a polymer backbone or a polymer branch comprises at least one monomer unit comprising

at least one pendant group or side group, that is, the monomer reactant from which the unit was obtained comprises at least three functional groups.

Examples of polyacids or polyesters that can be used for preparing an amorphous polyester resin include terephthalic acid, phthalic acid, isophthalic acid, fumaric acid, trimellitic acid, diethyl fumarate, dimethyl itaconate, cis-1,4-diacetoxy-2-butene, dimethyl fumarate, diethyl maleate, maleic acid, succinic acid, itaconic acid, succinic acid, cyclohexanoic acid, succinic anhydride, dodecylsuccinic acid, dodecylsuccinic anhydride, glutaric acid, glutaric anhydride, adipic acid, pimelic acid, suberic acid, azelaic acid, dodecanedioic acid, dimethyl naphthalenedicarboxylate, dimethyl terephthalate, diethyl terephthalate, dimethylisophthalate, diethylisophthalate, dimethylphthalate, phthalic anhydride, diethylphthalate, dimethylsuccinate, naphthalene dicarboxylic acid, dimer diacid, dimethylfumarate, dimethylmaleate, dimethylglutarate, dimethyladipate, dimethyl dodecylsuccinate, and combinations thereof. The organic polyacid or polyester reagent may be present, for example, in an amount from about 40 to about 60 mole % of the resin, in embodiments from about 42 to about 52 mole % of the resin, in embodiments from about 45 to about 50 mole % of the resin. Optionally a second polyacid can be used in an amount from about 0.1 to about 10 mole % of the resin.

Examples of polyols which may be used in generating an amorphous polyester resin include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanedimethanol, 1,3-cyclohexanedimethanol, xylenedimethanol, cyclohexanediol, diethylene glycol, bis(2-hydroxyethyl) oxide, dipropylene glycol, dibutylene glycol, and combinations thereof. The amount of organic polyol can vary, and may be present, for example, in an amount from about 40 to about 60 mole % of the resin, in embodiments from about 42 to about 55 mole % of the resin, in embodiments from about 45 to about 53 mole % of the resin. A second polyol can be used in an amount from about 0.1 to about 10 mole %, in embodiments, from about 1 to about 4 mole % of the resin.

Polycondensation catalysts may be used in forming the amorphous (or crystalline) polyester resin, and include tetraalkyl titanates, dialkyltin oxides, such as, dibutyltin oxide, tetraalkyltins, such as, dibutyltin dilaurate, and dialkyltin oxide hydroxides, such as, butyltin oxide hydroxide, aluminum alkoxides, alkyl zinc, dialkyl zinc, zinc oxide, stannous oxide, or combinations thereof. Such catalysts may be used in amounts of, for example, from about 0.01 mole % to about 5 mole % based on the starting polyacid or polyester reagent(s) used to generate the polyester resin.

In embodiments, the resin may be a crosslinkable resin. A crosslinkable resin is a resin including a crosslinkable group or groups such as a C=C bond or a pendant group or side group, such as, a carboxylic acid group. The resin can be crosslinked, for example, through a free radical polymerization with an initiator.

Examples of amorphous resins which may be used include alkali sulfonated-polyester resins, branched alkali sulfonated-polyester resins, alkali sulfonated-polyimide resins and branched alkali sulfonated-polyimide resins. Alkali sulfonated polyester resins may be useful in embodiments, such as, the metal or alkali salts of copoly(ethylene-terephthalate)-copolymers, copoly(ethylene-5-sulfo-isophthalate), copoly(propylene-terephthalate)-copolymers, copoly(propylene-5-sulfo-isophthalate), copoly(diethylene-terephthalate)-copolymers, copoly(propylene-5-sulfo-isophthalate), copoly(propylene-diethylene-terephthalate)-copolymers, copoly(propylene-butylene-terephthalate)-copolymers, copoly(propylene-5-sulfo-isophthalate), copoly(propoxylated bisphenol-A-fumarate)-copolymers, copoly(ethoxylated bisphenol-A-5-sulfo-isophthalate), copoly(ethoxylated bisphenol-A-5-sulfo-isophthalate), and copoly(ethoxylated bisphenol-A-maleate)-copolymers, copoly(ethoxylated bisphenol-A-5-sulfo-isophthalate), wherein the alkali metal is, for example, a sodium, a lithium or a potassium ion.

In embodiments, an unsaturated amorphous polyester resin may be used as a latex resin, such as, those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate) and combinations thereof.

In embodiments, a suitable amorphous resin may include alkoxylated bisphenol A fumarate/terephthalate-based polyester and copolyester resins. In embodiments, a suitable polyester resin may be an amorphous polyester resin, such as, a poly(propoxylated bisphenol A co-fumarate) resin. Examples of such resins and processes for production thereof include those disclosed in U.S. Pat. No. 6,063,827, the disclosure of which is hereby incorporated by reference in entirety.

An example of a linear propoxylated bisphenol A fumarate resin is available under the trade name SPARII from Resana S/A Industrias Quimicas, Sao Paulo Brazil. Other propoxylated bisphenol A fumarate resins that are commercially available include GTUF and FPESL-2 from Kao Corporation, Japan, and EM181635 from Reichhold, Research Triangle Park, N.C., and the like.

In embodiments, a resin may comprises plural species of amorphous resins, such as, one or more high molecular weight amorphous resins, one or more low molecular weight amorphous resins, or a combination thereof. The relative amounts of the different species of amorphous resins is a design choice.

For forming a crystalline polyester resin, suitable organic polyols include aliphatic polyols with from about 2 to about 36 carbon atoms, such as 1,2-ethanediol, 1,3-propanediol, 1,4-butanediol, 1,5-pentanediol, 2,2-dimethylpropane-1,3-diol, 1,6-hexanediol, 1,7-heptanediol, 1,8-octanediol, 1,9-nonenediol, 1,10-decanediol, 1,12-dodecanediol and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like, including their structural isomers. The aliphatic polyol may be, for example, selected in an amount from about 40 to about 60 mole %, in embodiments from about 42 to about 55 mole %, in embodiments from about 45 to about 53 mole %. A second polyol can be used in an amount from about 0.1 to about 10 mole %, in embodiments from about 1 to about 4 mole % of the resin.

Examples of organic polyacid or polyester reagents for preparing a crystalline resin include oxalic acid, succinic acid, glutaric acid, adipic acid, suberic acid, azelaic acid, sebatic acid, fumaric acid, dimethyl fumarate, dimethyl itaconate, cis, 1,4-diacetoxy-2-butene, diethyl fumarate, diethyl maleate, phthalic acid, isophthalic acid, terephthalic acid, naphthalene-2,6-dicarboxylic acid, naphthalene-2,7-dicarboxylic acid, cyclohexane dicarboxylic acid (sometimes referred to herein, in embodiments, as cyclohexanedioic acid), malonic acid and mesaconic acid, a polyester or anhydride thereof; and an alkali sulfo-organic polyacid, such as, the sodio, lithio or potassio salt of dimethyl-5-sulfo-isophthalate, dialkyl-5-sulfo-isophthalate-4-sulfo-1,8-naphthalic anhydride, 4-sulfo-phthalic acid, dimethyl-4-sulfo-phthalate, dialkyl-4-sulfo-phthalate, 4-sulfophenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfo-p-hydroxybenzoic acid, N,N-bis(2-hydroxyethyl)-2-amino ethane sulfonate, or mixtures thereof. The organic polyacid may be selected in an amount of, for example, in embodiments from about 40 to about 60 mole %, in embodiments from about 42 to about 52 mole %, in embodiments from about 45 to about 50 mole %. Optionally, a second polyacid can be used in an amount from about 0.1 to about 10 mole % of the resin.

lene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipatenonylene-decanoate), poly(octylene-adipate), and so on, wherein alkali is a metal like sodium, lithium or potassium. Examples of polyamides include poly(ethylene-adipamide), poly(propylene-adipamide), poly(butylenes-adipamide), poly(pentylene-adipamide), poly(hexylene-adipamide), poly(octylene-adipamide), poly(ethylene-succinimide), and poly(propylene-sebacamide). Examples of polyimides include poly(ethylene-adipimide), poly(propylene-adipimide), poly(butylene-adipimide), poly(pentylene-adipimide), poly(hexylene-adipimide), poly(octylene-adipimide), poly(ethylene-succinimide), poly(propylene-succinimide), and poly(butylene-succinimide).

Suitable crystalline resins which may be utilized, optionally in combination with an amorphous resin as described above, include those disclosed in U.S. Pub. No. 2006/0222991, the disclosure of which is hereby incorporated by reference in entirety.

In embodiments, a suitable crystalline resin may include a resin formed of ethylene glycol and a mixture of dodecanedioic acid and fumaric acid comonomers.

The crystalline resin may be present, for example, in an amount from about 1 to about 85% by weight of the toner components, in embodiments from about 2 to about 50% by weight of the toner components, in embodiments from about 5 to about 15% by weight of the toner components. The crystalline resin can possess various melting points of, for example, from about 30° C. to about 120° C., in embodiments from about 50° C. to about 90° C., in embodiments from about 60° C. to about 80° C. The crystalline resin may have a number average molecular weight ( $M_n$ ), as measured by gel permeation chromatography (GPC) of, for example, from about 1,000 to about 50,000, in embodiments from about 2,000 to about 25,000, and a weight average molecular weight ( $M_w$ ) of, for example, from about 2,000 to about 100,000, in embodiments from about 3,000 to about 80,000, as determined by GPC using polystyrene standards. The molecular weight distribution ( $M_w/M_n$ ) of the crystalline resin may be, for example, from about 2 to about 6, in embodiments from about 3 to about 4.

Examples of other suitable resins or polymers which may be utilized in forming a toner include, but are not limited to, poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), poly(styrene-butyl acrylate-acrylonitrile-acrylic acid), and combinations thereof. The polymer may be, for example, block, random, or alternating copolymers.

## b. Catalyst

Condensation catalysts which may be used in the polyester reaction include tetraalkyl titanates; dialkyltin oxides, such as, dibutyltin oxide; tetraalkyltins, such as, dibutyltin dilaurate; dibutyltin diacetate; dibutyltin oxide; dialkyltin oxide hydroxides, such as, butyltin oxide hydroxide; aluminum alkoxides, alkyl zinc, dialkyl zinc, zinc oxide, stannous oxide, stannous chloride, butylstannoic acid or combinations thereof.

Such catalysts may be used in amounts of, for example, from about 0.01 mole % to about 5 mole % based on the amount of starting polyacid, polyol or polyester reagent in the reaction mixture.

Generally, as known in the art, the polyacid/polyester and polyols reagents, are mixed together, optionally with a catalyst, and incubated at an elevated temperature, such as, from about 180° C. or more, from about 190° C. or more, from about 200° C. or more, and so on, which can be conducted anaerobically, to enable esterification to occur until equilibrium, which generally yields water or an alcohol, such as, methanol, arising from forming the ester bonds in esterification reactions. The reaction can be conducted under vacuum to promote polymerization.

Branching agents can be used, and include, for example, a multivalent polyacid such as 1,2,4-benzene-tricarboxylic acid, 1,2,4-cyclohexanetricarboxylic acid, 2,5,7-naphthalenetricarboxylic acid, 1,2,4-naphthalenetricarboxylic acid, 1,2,5-hexanetricarboxylic acid, 1,3-dicarboxyl-2-methyl-2-methylene-carboxylpropane, tetra(methylene-carboxyl)methane, 1,2,7,8-octanetetracarboxylic acid, acid anhydrides thereof, lower alkyl esters thereof and so on. The branching agent can be used in an amount from about 0.01 to about 10 mole % of the resin, from about 0.05 to about 8 mole % or from about 0.1 to about 5 mole % of the resin.

It may be desirable to crosslink the polymer. A suitable resin conducive to crosslinking is one with a reactive group, such as, a C=C bond or with pendant or side groups, such as, a carboxylic acid group. The resin can be crosslinked, for example, through free radical polymerization with an initiator. Suitable initiators include peroxides such as, organic peroxides or azo compounds, for example diacyl peroxides, such as, decanoyl peroxide, lauroyl peroxide and benzoyl peroxide, ketone peroxides, such as, cyclohexanone peroxide and methyl ethyl ketone, alkyl peroxy esters, such as, t-butyl peroxy neodecanoate, 2,5-dimethyl 2,5-di(2-ethyl hexanoyl peroxy)hexane, t-amyl peroxy 2-ethyl hexanoate, t-butyl peroxy 2-ethyl hexanoate, t-butyl peroxy acetate, t-amyl peroxy acetate, t-butyl peroxy benzoate, t-amyl peroxy benzoate, alkyl peroxides, such as, dicumyl peroxide, 2,5-dimethyl 2,5-di(t-butyl peroxy)hexane, t-butyl cumyl peroxide, bis(t-butyl peroxy)diisopropyl benzene, di-t-butyl peroxide and 2,5-dimethyl 2,5-di(t-butyl peroxy)hexyne-3, alkyl hydroperoxides, such as, 2,5-dihydro peroxy 2,5-dimethyl hexane, cumene hydroperoxide, t-butyl hydroperoxide and t-amyl hydroperoxide, and alkyl peroxyketals, such as, n-butyl 4,4-di(t-butyl peroxy)valerate, 1,1-di(t-butyl peroxy) 3,3,5-trimethyl cyclohexane, 1,1-di(t-butyl peroxy)cyclohexane, 1,1-di(t-amyl peroxy)cyclohexane, 2,2-di(t-butyl peroxy)butane, ethyl 3,3-di(t-butyl peroxy)butyrate and ethyl 3,3-di(t-amyl peroxy)butyrate, azobis-isobutyronitrile, 2,2'-azobis(isobutyronitrile), 2,2'-azobis(2,4-dimethyl valeronitrile), 2,2'-azobis(methyl butyronitrile), 1,1'-azobis(cyano cyclohexane), 1,1-di(t-butyl peroxy)-3,3,5-trimethylcyclohexane, combinations thereof and the like. The amount of initiator used is proportional to the degree of crosslinking desired, and thus, the gel content of the polyester material. The amount of initiator used may range from, for example, about 0.01 to

about 10 weight %, or from about 0.1 to about 5 weight % of the polyester resin. In the crosslinking, it is desirable that substantially all of the initiator be consumed. The crosslinking may be carried out at high temperature, and thus the reaction may be very fast, for example, less than 10 minutes, such as from about 20 seconds to about 2 minutes residence time.

Polyester resins suitable for use in an imaging device are those which carry one or more properties, such as, a  $T_g$  (onset) of at least about 40° C., at least about 45° C., at least about 50° C., at least about 55° C.; a  $T_s$  of at least about 110° C., at least about 115° C., at least about 120° C., at least about 125° C.; an acid value (AV) of at least about 10, at least about 12.5, at least about 15, at least about 17.5; and an  $M_w$  of at least about 5000, at least about 15,000, at least about 20,000, at least about 100,000.

## 2. Colorants

Suitable colorants include those comprising carbon black, such as, REGAL 330® and Nipex 35; magnetites, such as, Mobay magnetites, MO8029™ and MO8060™; Columbian magnetites, MAPICO® BLACK; surface-treated magnetites; Pfizer magnetites, CB4799™, CB5300™, CB5600™ and MCX6369™; Bayer magnetites, BAYFEROX 8600™ and 8610™; Northern Pigments magnetites, NP-604™ and NP-608™; Magnox magnetites, TMB-100™ or TMB-104™; and the like.

Colored pigments, such as, cyan, magenta, yellow, red, orange, green, brown, blue or mixtures thereof can be used. The additional pigment or pigments can be used as water-based pigment dispersions.

Examples of pigments include SUNSPERSE 6000, FLEXIVERSE and AQUATONE, water-based pigment dispersions from SUN Chemicals; HELIOGEN BLUE L6900™, D6840™, D7080™, D7020™, PYLAM OIL BLUE™, PYLAM OIL YELLOW™ and PIGMENT BLUE I™ available from Paul Uhlrich & Company, Inc.; PIGMENT VIOLET I™, PIGMENT RED 48™, LEMON CHROME YELLOW DCC 1026™, TOLUIDINE RED™ and BON RED CTM available from Dominion Color Corporation, Ltd., Toronto, Ontario; NOVAPERMYELLOW FGL™ and HOSTAPERM PINK ETM from Hoechst; CINQUASIA MAGENTA™ available from E.I. DuPont de Nemours & Co., and the like.

Examples of magenta pigments include 2,9-dimethyl-substituted quinacridone, an anthraquinone dye identified in the Color Index as CI 60710, CI Dispersed Red 15, a diazo dye identified in the Color Index as CI 26050, CI Solvent Red 19 and the like.

Illustrative examples of cyan pigments include copper tetra(octadecylsulfonamido) phthalocyanine, a copper phthalocyanine pigment listed in the Color Index as CI 74160, CI Pigment Blue, Pigment Blue 15:3, Pigment Blue 15:4, an Anthrazine Blue identified in the Color Index as CI 69810, Special Blue X-2137 and the like.

Illustrative examples of yellow pigments are diarylide yellow 3,3-dichlorobenzidene acetocetanilide, a monoazo pigment identified in the Color Index as CI 12700, CI Solvent Yellow 16, a nitrophenyl amine sulfonamide identified in the Color Index as Foron Yellow SE/GLN, CI Disperse Yellow 3, 2,5-dimethoxy-4-sulfonanilide phenylazo-4'-chloro-2,5-dimethoxy acetocetanilide and Permanent Yellow FGL.

Other known colorants can be used, such as, Levanyl Black A-SF (Miles, Bayer) and Sunperse Carbon Black LHD 9303 (Sun Chemicals), and colored dyes, such as, Neopen Blue (BASF), Sudan Blue OS (BASF), PV Fast Blue B2G 01 (American Hoechst), Sunperse Blue BHD 6000 (Sun Chemicals), Irgalite Blue BCA (CibaGeigy), Paliogen Blue

6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), SUCD-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing and the like. Other pigments that can be used, and which are commercially available include various pigments in the color classes, Pigment Yellow 74, Pigment Yellow 14, Pigment Yellow 83, Pigment Orange 34, Pigment Red 238, Pigment Red 122, Pigment Red 48:1, Pigment Red 269, Pigment Red 53:1, Pigment Red 57:1, Pigment Red 83:1, Pigment Violet 23, Pigment Green 7 and so on, and combinations thereof.

The colorant, for example carbon black, cyan, magenta and/or yellow colorant, may be incorporated in an amount sufficient to impart the desired color to the toner. In general, pigment or dye, the total amount of colorant may be employed in a total amount ranging from about 2% to about 60% by weight of the toner particles on a solids basis, from about 3% to about 55% by weight, from about 4% to about 45% by weight, from about 4.5% to about 40%, from about 5% to about 40% by weight of the toner particles. As provided herein, the total amount of colorant is divided into n portions, wherein n is 2, 3, 4, 5 or more, and the portions can be of the same size or amount. As also provided herein, the colorants can be the same or different color, and can be the same or different particular pigment. In embodiments, one or more colorants are added continuously to the toner particle reaction mixture.

In embodiments, more than one colorant may be present in a toner particle. For example, two colorants, three colorants or more may be present in a toner particle, such as a black and a cyan. For example, a first colorant of pigment blue, may be present in an amount ranging from about 2% to about 10% by weight of the toner particle on a solids basis, from about 3% to about 8% by weight or from about 5% to about 10% by weight; with a second colorant of pigment yellow that may be present in an amount ranging from about 5% to about 20% by weight of the toner particle on a solids basis, from about 6% to about 15% by weight or from about 10% to about 20% by weight and so on.

In embodiments, the ratio of the first colorant to the second colorant, when present, on a weight basis, can range from about 1:20 to 1:2 or 1:1. Hence, the first colorant can be present at a weight ratio of 1:15, 1:10, 1:7, 1:5, 1:4 and so on relative to the second colorant. In other embodiments, the ratio of the second colorant, when present, to the first colorant, on a weight basis, can range from about 1:20 to 1:2 or 1:1. Hence, the second colorant can be present at a weight ratio of 1:15, 1:10, 1:7, 1:5, 1:4 and so on relative to the first colorant.

In embodiments, the ratio of the first colorant to the third colorant, on a weight basis, can range from about 5:1 to 1:1 to

1:5. Hence, the first colorant can be present at a weight ratio of 4:1, 3:1, 1:2, 1:4, 1:5 and so on relative to the third colorant. In other embodiments, the ratio of the second colorant, when present, to the fourth colorant, when present, on a weight basis, can range from about 3:1 to 1:1 to 1:3. Hence, the second colorant can be present at a weight ratio of 2:1, 1.5:1, 1:2, 1:2.5 and so on relative to the fourth colorant.

In embodiments, the ratio of the total amount of the first and when present, third colorant, to the total of the second and 10 when present, fourth colorant can be about 30:1 to about 1:30, from about 25:1 to about 1:5, from about 20:1 to about 1:1, from about 15:1 to about 2:1 and so on. However, essentially any ratio can be used as a design choice to obtain a color of interest.

15 In embodiments, the first and the third colorants and the same, and hence, the colorant is added to the particle reaction mixture in portions. In other embodiments, different pigments of a particular color are added in the different portions. Hence, for example, two different black pigments can be 20 added at the different times during particle formation and aggregation. Similarly, one colorant can be added just once in the process, or when added in plural portions, the same or different colorants can be used, and the amounts of each portion can be the same or different.

### 3. Optional Components

#### a. Surfactants

In embodiments, toner compositions may be in dispersions including surfactants. Emulsion aggregation methods where the polymer and other components of the toner are in combination can employ one or more surfactants to form an emulsion.

30 One, two or more surfactants may be used. The surfactants may be selected from ionic surfactants and nonionic surfactants, or combinations thereof. Anionic surfactants and cationic surfactants are encompassed by the term, "ionic surfactants."

In embodiments, the surfactant or the total amount of surfactants may be used in an amount of from about 0.01% to 40 about 5% by weight of the toner-forming composition, for example, from about 0.75% to about 4% by weight of the toner-forming composition, in embodiments, from about 1% to about 3% by weight of the toner-forming composition.

45 Examples of nonionic surfactants include, for example, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether and dialkylphenoxy poly(ethyleneoxy) ethanol, for example, available from Rhone-Poulenc as IGEPAL CA-210<sup>TM</sup>, IGEPAL CA-520<sup>TM</sup>, IGEPAL CA-720<sup>TM</sup>, IGEPAL CO-890<sup>TM</sup>, IGEPAL CO-720<sup>TM</sup>, IGEPAL CO-290<sup>TM</sup>, IGEPAL CA-210<sup>TM</sup>, ANTAROX 890<sup>TM</sup> and ANTAROX 897<sup>TM</sup>. Other examples of suitable nonionic surfactants include a block copolymer of polyethylene oxide 55 and polypropylene oxide, including those commercially available as SYNPERONIC<sup>®</sup> PR/F, in embodiments, SYNPERONIC<sup>®</sup> PR/F 108; and a DOWFAX, available from The Dow Chemical Corp.

Anionic surfactants include sulfates and sulfonates, such 60 as, sodium dodecylsulfate (SDS), sodium dodecylbenzene sulfonate, sodium dodecylnaphthalene sulfate and so on; dialkyl benzenealkyl sulfates; acids, such as, palmitic acid, and NEOGEN or NEOGEN SC obtained from Daiichi Kogyo Seiyaku, and so on, combinations thereof and the like. Other 65 suitable anionic surfactants include, in embodiments, alkyl-diphenyloxide disulfonates or TAYCA POWER BN2060 from Tayca Corporation (Japan), which is a branched sodium

dodecyl benzene sulfonate. Combinations of those surfactants and any of the foregoing nonionic surfactants may be used in embodiments.

Examples of cationic surfactants include, for example, alkylbenzyl dimethyl ammonium chloride, dialkyl benzene-alkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, trimethyl ammonium bromides, halide salts of quarternized polyoxyethylalkylamines, dodecylbenzyl triethyl ammonium chlorides, MIRAPOL® and ALKAQUAT® available from Alkaril Chemical Company, SANISOL® (benzalkonium chloride) available from Kao Chemicals and the like, and mixtures thereof, including, for example, a nonionic surfactant as known in the art or provided hereinabove.

b. Waxes

The toners of the instant disclosure, optionally, may contain a wax, which can be either a single type of wax or a mixture of two or more different types of waxes (hereinafter identified as, "a wax"). A wax can be added to a toner formulation or to a developer formulation, for example, to improve particular toner properties, such as, toner particle shape, charging, fusing characteristics, gloss, stripping, offset properties and the like. Alternatively, a combination of waxes can be added to provide multiple properties to a toner or a developer composition. A wax may be included as, for example, a fuser roll release agent.

The wax may be combined with the resin-forming composition for forming toner particles. When included, the wax may be present in an amount of, for example, from about 1 wt % to about 25 wt % of the toner particles, in embodiments, from about 5 wt % to about 20 wt % of the toner particles.

Waxes that may be selected include waxes having, for example, a weight average molecular weight of from about 500 to about 20,000, in embodiments, from about 1,000 to about 10,000. Waxes that may be used include, for example, polyolefins, such as, polyethylene, polypropylene and polybutene waxes, such as, those that are commercially available, for example, POLYWAX™ polyethylene waxes from Baker Petrolite, wax emulsions available from Michaelman, Inc. or Daniels Products Co., EPOLENE N15™ which is commercially available from Eastman Chemical Products, Inc., VISCOL 550-PTM, a low weight average molecular weight polypropylene available from Sanyo Kasei K.K.; plant-based waxes, such as carnauba wax, rice wax, candelilla wax, sumac wax and jojoba oil; animal-based waxes, such as beeswax; mineral-based waxes and petroleum-based waxes, such as montan wax, ozokerite, ceresin wax, paraffin wax, micro-crystalline wax and Fischer-Tropsch waxes; ester waxes obtained from higher fatty acids and higher alcohols, such as stearyl stearate and behenyl behenate; ester waxes obtained from higher fatty acids and monovalent or multivalent lower alcohols, such as butyl stearate, propyl oleate, glyceride monostearate, glyceride distearate and pentaerythritol tetra-behenate; ester waxes obtained from higher fatty acids and multivalent alcohol multimers, such as diethyleneglycol monostearate, dipropylene glycol distearate, diglyceryl distearate and triglyceryl tetras Stearate; sorbitan higher fatty acid ester waxes, such as sorbitan monostearate; cholesterol higher fatty acid ester waxes, such as, cholesteryl stearate, and so on.

Examples of functionalized waxes that may be used include, for example, amines and amides, for example, AQUA SUPERSLIP 6550™ and SUPERSLIP 6530™ available from Micro Powder Inc.; fluorinated waxes, for example, POLYFLUO 190™, POLYFLUO 200™, POLYSILK 19™

and POLYSILK 14™ available from Micro Powder Inc.; mixed fluorinated amide waxes, for example, MICROSPERSION 19™ also available from Micro Powder Inc.; imides, esters, quaternary amines, carboxylic acids, acrylic polymer emulsions, for example, JONCRYL 74™, 89™, 130™, 537™ and 538™ available from SC Johnson Wax; and chlorinated polypropylenes and polyethylenes available from Allied Chemical, Petrolite Corp. and SC Johnson. Mixtures and combinations of the foregoing waxes also may be used in embodiments.

c. Aggregating Factor (Flocculant)

An aggregating factor or flocculant optionally may be used and may be an inorganic cationic coagulant, such as, for example, polyaluminum chloride (PAC), polyaluminum sulfosilicate (PASS), aluminum sulfate, zinc sulfate, magnesium sulfate and chlorides of magnesium, calcium, zinc, beryllium, aluminum, sodium, other metal halides including monovalent and divalent halides.

The aggregating factor may be present in an emulsion in an amount of from, for example, from about 0.01 wt % to about 10 wt %, from about 0.05 to about 5 wt %, from about 1 to about 4 wt %, from about 2 to about 3 wt %, based on the total solids in the toner.

The aggregating factor may also contain minor amounts of other components, for example, nitric acid.

In embodiments, a sequestering agent or chelating agent may be introduced after aggregation is complete to sequester or to extract a metal complexing ion, such as, aluminum, from the aggregation process. Thus, the sequestering, chelating or complexing agent used after aggregation is complete may comprise an organic complexing component, such as, ethylenediaminetetraacetic acid (EDTA), gluconal, hydroxyl-2, 2'iminodisuccinic acid (HIDS), dicarboxylmethyl glutamic acid (GLDA), methyl glycidyl diacetic acid (MGDA), hydroxydiethyliminodiacetic acid (HIDA), sodium gluconate, potassium citrate, sodium citrate, nitrotriacetate salt, humic acid, fulvic acid; salts of EDTA, such as, alkali metal salts of EDTA, tartaric acid, gluconic acid, oxalic acid, polyacrylates, sugar acrylates, citric acid, polyaspartic acid, diethylenetriamine pentaacetate, 3-hydroxy-4-pyridinone, dopamine, eucalyptus, iminodisuccinic acid, ethylenediaminedisuccinate, polysaccharide, sodium ethylenedinitrilotetraacetate, thiamine pyrophosphate, farnesyl pyrophosphate, 2-aminoethylpyrophosphate, hydroxyl ethylidene-1, 1-diphosphonic acid, aminotrimethylene phosphonic acid, diethylene triaminepentamethylene phosphonic acid, ethylenediamine tetramethylene phosphonic acid, and mixtures thereof.

d. Surface Additive

In embodiments, the toner particles can be mixed with one or more of silicon dioxide or silica ( $\text{SiO}_2$ ), titania or titanium dioxide ( $\text{TiO}_2$ ) and/or cerium oxide. Silica may be a first silica and a second silica. The second silica may have a larger average size (diameter) than the first silica. The first silica may have an average primary particle size, measured in diameter, in the range of, for example, from about 5 nm to about 50 nm, such as, from about 5 nm to about 25 nm or from about 20 nm to about 40 nm. The second silica may have an average primary particle size, measured in diameter, in the range of, for example, from about 100 nm to about 200 nm, such as, from about 100 nm to about 150 nm or from about 125 nm to about 145 nm. The titania may have an average primary particle size in the range of, for example, about 5 nm to about 50 nm, such as, from about 5 nm to about 20 nm or from about 10 nm to about 50 nm. The cerium oxide may have an average primary particle size in the range of, for example, about 5 nm

## 15

to about 50 nm, such as, from about 5 nm to about 20 nm or from about 10 nm to about 50 nm.

Zinc stearate also may be used as an external additive, for example, as a lubricant. Calcium stearate and magnesium stearate may provide similar functions. Zinc stearate may have an average primary particle size in the range of, for example, from about 500 nm to about 700 nm, such as, from about 500 nm to about 600 nm or from about 550 nm to about 650 nm.

## e. Carrier

Carrier particles include those that are capable of triboelectrically obtaining a charge of polarity opposite to that of the toner particles. Illustrative examples of suitable carrier particles include granular zircon, granular silicon, glass, steel, nickel, ferrites, iron ferrites, silicon dioxide, nickel berry carriers as disclosed in U.S. Pat. No. 3,847,604, the entire disclosure of which is hereby incorporated herein by reference, comprised of nodular carrier beads of nickel, characterized by surfaces of reoccurring recesses and protrusions thereby providing particles with a relatively large external area, those disclosed in U.S. Pat. Nos. 4,937,166 and 4,935,326, the disclosures of which are hereby incorporated herein by reference, and so on. In embodiments, the carrier particles may have an average particle size of, for example, from about 20 to about 85  $\mu\text{m}$ , such as, from 30 to about 60  $\mu\text{m}$ , or from about 35 to about 50  $\mu\text{m}$ .

## B. Toner Particle Preparation

## 1. Method

## a. Resin Emulsion Particle Formation

The toner particles may be prepared by any method within the purview of one skilled in the art, for example, any of the emulsion/aggregation methods can be used with a resin, such as, a polyester resin so long as total pigment is introduced into the developing particle in graded amounts and at different times, that is, portions of the total pigment are added at different times during toner particle development.

In embodiments relating to an emulsification/aggregation process, a resin can be dissolved in a solvent, and can be mixed into an emulsion medium, for example water, such as, deionized water, optionally containing a stabilizer, and optionally a surfactant. Examples of suitable stabilizers include water-soluble alkali metal hydroxides, such as, sodium hydroxide, potassium hydroxide, lithium hydroxide, beryllium hydroxide, magnesium hydroxide, calcium hydroxide or barium hydroxide; ammonium hydroxide; alkali metal carbonates, such as, sodium bicarbonate, lithium bicarbonate, potassium bicarbonate, lithium carbonate, potassium carbonate, sodium carbonate, beryllium carbonate, magnesium carbonate, calcium carbonate, barium carbonate or cesium carbonate; or mixtures thereof. When a stabilizer is used, the stabilizer can be present in amounts of from about 0.1% to about 5%, from about 0.5% to about 3% by weight of the resin. When such salts are added to the composition as a stabilizer, in embodiments, incompatible metal salts are not present in the composition, for example, a composition can be completely or essentially free of zinc and other incompatible metal ions, for example, Ca, Fe, Ba etc., that form water-insoluble salts. The term "essentially free" refers, for example, to the incompatible metal ions as present at a level of less than about 0.01%, less than about 0.005% or less than about 0.001%, by weight of the wax and resin. The stabilizer can be added to the mixture at ambient temperature, or can be heated to the mixture temperature prior to addition.

Optionally, a surfactant may be added to the aqueous emulsion medium, for example, to afford additional stabilization

## 16

to the resin or to enhance emulsification of the resin. Suitable surfactants include anionic, cationic and nonionic surfactants as taught herein.

Thus, a toner composition may be prepared by preparing a mixture of a resin emulsion, a first colorant or colorant dispersion, optionally, a second colorant or colorant dispersion, an optional wax or a wax dispersion and any other desired reagents, optionally, with surfactants as described above to form a toner reaction mixture, generally in the form of an emulsion. The pH of the mixture may be adjusted as needed with an acid, such as, for example, acetic acid, nitric acid or the like. The colorants optionally can be added in portions to the above mixture of can be added continuously during mixing of the reagents and early particle formation.

## 15 b. Aggregation

Early particle formation can occur in the presence of an aggregating factor. Suitable aggregating factors include, for example, aqueous solutions of a divalent cation, a multivalent cation or a compound comprising same, a polyaluminum halide, such as, polyaluminum chloride (PAC) or the corresponding bromide, fluoride or iodide; a polyaluminum silicate, such as, polyaluminum sulfosilicate (PASS); or a water soluble metal salt, including, aluminum chloride, aluminum nitrite, aluminum sulfate, potassium aluminum sulfate, calcium acetate, calcium chloride, calcium nitrite, calcium oxydate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate or combinations thereof.

30 In embodiments, the aggregating factor may be added to the mixture at a temperature that is below the glass transition temperature ( $T_g$ ) of the resin or of a polymer.

The aggregating factor may be added to the mixture components to form a toner in an amount of, for example, from 35 about 0.1 part per hundred (pph) to about 5 pph, in embodiments, from about 0.2 pph to about 0.3 pph, in embodiments, from about 0.3 pph to about 2 pph of the reaction mixture. The aggregating factor can be added while the mixture is homogenized or stirred. Mixing can be at a speed of about 600 rpm 40 to about 4,000 rpm, in embodiments, from about 700 rpm to about 3,000 rpm, using for example, an IKA ULTRA TUR-RAX T50 probe homogenizer.

The temperature or the mixture can be below the  $T_g$  of the resin or polymer, in embodiments, from about 30° C. to about 45 90° C., in embodiments, from about 35° C. to about 70° C. The growth and shaping of the particles following addition of the aggregation factor may be accomplished under any suitable condition(s).

As provided herein, the aggregating factor is introduced 50 when the original toner reaction mixture is prepared, including addition of first and optional second colorant, rather added in portions or continuously. Hence, the aggregating factor is added to generate pre-aggregated toner particles after the pH of the mixture is adjusted as taught herein while the mixture is being stirred.

The particles are permitted to aggregate until a predetermined desired pre-aggregated toner particle size is obtained, with the size determined, for example, with a Coulter Counter. Then, the third colorant, along with an optional 60 fourth colorant or colorant dispersion, are added to the mixture, either in portions or continuously, which is then incubated further to form the core particle. Aggregation is permitted to occur, for example, by raising the temperature or maintaining the mixture at an elevated temperature. A suitable particle size can be less than about 4  $\mu\text{m}$ , less than about 3.5  $\mu\text{m}$ , less than about 3  $\mu\text{m}$ , less than about 2.5  $\mu\text{m}$ , for 65 example, and at that time, the second aliquot of colorant(s) is

added to the emulsion. Following addition of the remainder of the colorant(s), the incubation is continued for additional particle growth.

In embodiments, the total amount of a colorant is introduced in a portion, two portions, three portions, four portions or more, or a colorant can be introduced continuously during aggregation. All portions can be of the same amount of colorant, or the amounts may vary across the portions as a design choice. Thus, colorant amounts can progress in amount over aggregation, can decrease in amount over aggregation, can be higher at the beginning with the other portions of equal amount, can be higher at the last introduction of colorant with the other portions of equal amount and so on. For example, when a colorant is added in a first and second portion, the amount of the first and the second portions, as a ratio by weight, can be 1:9, 1:8, 1:7, 1:6, 1:5, 1:4, 1:3, 1:2, 1:1; 2:1, 3:1, 4:1, 5:1, 6:1, 7:1, 8:1 or 9:1, for example. Other ratios can be used as well, as a design choice. Essentially the same ratios can apply to the first and third colorants. Essentially the same ratios can apply to the second and fourth colorants. In embodiments, more than four colorants can be used, that is, five colorants, six colorants, seven colorants or more can be used in a toner.

The aggregation thus may proceed by maintaining the mixture, for example, at elevated temperature, or slowly raising the temperature, for example, from about 30° C. to about 80° C., and holding the mixture at that temperature for from about 0.5 hours to about 6 hours, in embodiments, from about hour 1 to about 5 hours, while maintaining stirring, to provide the desired aggregated particles. Once the predetermined desired particle size is attained, the growth process is halted.

The characteristics of the toner particles may be determined by any suitable technique and apparatus. Volume average particle diameter and geometric standard deviation may be measured using an instrument, such as, a Beckman Coulter Multisizer 3, operated in accordance with the instructions of the manufacturer. Representative sampling may occur by taking a sample, filtering through a 25  $\mu\text{m}$  membrane, diluting in an isotonic solution to obtain a concentration of about 10% and then reading the sample, for example, in a Beckman Coulter Multisizer 3.

The growth and shaping may be conducted under conditions in which aggregation occurs separate from coalescence. For separate aggregation and coalescence stages, the aggregation process may be conducted under shearing conditions at an elevated temperature, for example, of from about 30° C. to about 80° C., in embodiments, from about 35° C. to about 70° C., which may be below the  $T_g$  of the resin or a polymer.

In embodiments, the aggregate particles may be of a size of less than about 6  $\mu\text{m}$ , in embodiments from about 4  $\mu\text{m}$  to about 5.5  $\mu\text{m}$ , in embodiments from about 4.5  $\mu\text{m}$  to about 5  $\mu\text{m}$ .

In embodiments, after aggregation, but prior to coalescence, a resin coating may be applied to the aggregated particles to form a shell thereover. Any resin described herein or as known in the art may be used as the shell. In embodiments, an amorphous polyester resin latex as described herein may be included in the shell. In embodiments, an amorphous polyester resin latex described herein may be combined with a different resin, and then added to the particles as a resin coating to form a shell. In embodiments, the shell can comprise one or more colorants.

A shell resin may be applied to the aggregated particles by any method within the purview of those skilled in the art. In embodiments, the resins used to form the shell may be in an emulsion, optionally including any surfactant described

herein. The emulsion possessing the resins may be combined with the aggregated particles so that the shell forms over the aggregated particles.

The formation of the shell over the aggregated particles may occur while heating to a temperature from about 30° C. to about 80° C., in embodiments, from about 35° C. to about 70° C. The formation of the shell may take place for a period of time from about 5 minutes to about 10 hours, in embodiments from about 10 minutes to about 5 hours.

10 The shell may be present in an amount from about 1% by weight to about 80% by weight of the toner components, in embodiments from about 10% by weight to about 40% by weight of the toner components, in embodiments from about 20% by weight to about 35% by weight of the toner components.

c. Coalescence

Following aggregation to a desired particle size and application of any optional shell, the particles then may be coalesced to a desired final shape, such as, a circular shape, for example, to correct for irregularities in shape and size, the coalescence being achieved by, for example, heating the mixture to a temperature from about 45° C. to about 100° C., in embodiments from about 55° C. to about 99° C., which may be at or above the  $T_g$  of the resins used to form the toner particles, and/or reducing the stirring, for example to from about 1000 rpm to about 100 rpm, in embodiments from about 800 rpm to about 200 rpm. Coalescence may be conducted over a period from about 0.01 to about 9 hours, in embodiments from about 0.1 to about 4 hours, see, for example, U.S. Pat. No. 7,736,831.

30 Optionally, a coalescing agent can be used. Examples of suitable coalescence agents include, but are not limited to, benzoic acid alkyl esters, ester alcohols, glycol/ether-type solvents, long chain aliphatic alcohols, aromatic alcohols, mixtures thereof and the like. Examples of benzoic acid alkyl esters include those where the alkyl group, which can be straight or branched, substituted or unsubstituted, has from about 2 to about 30 carbon atoms, such as decyl or isodecyl benzoate, nonyl or isononyl benzoate, octyl or isoctyl benzoate, 2-ethylhexyl benzoate, tridecyl or isotridecyl benzoate, 3,7-dimethyloctyl benzoate, 3,5,5-trimethylhexyl benzoate, mixtures thereof and the like. Examples of such benzoic acid alkyl esters include VELTA® 262 (isodecyl benzoate) and VELTA® 368 (2-ethylhexyl benzoate) available from Velsicol Chemical Corp. Examples of ester alcohols include hydroxylalkyl esters of alkanoic acids, where the alkyl group, which can be straight or branched, substituted or unsubstituted, and can have from about 2 to about 30 carbon atoms, such as, 2,2,4-trimethylpentane-1,3-diol monoisobutyrate.

40 An example of an ester alcohol is TEXANOL® (2,2,4-trimethylpentane-1,3-diol monoisobutyrate) available from Eastman Chemical Co. Examples of glycol/ether-type solvents include diethylene glycol monomethylether acetate, diethylene glycol monobutylether acetate, butyl carbitol acetate (BCA) and the like. Examples of long chain aliphatic alcohols include those where the alkyl group is from about 5 to about 20 carbon atoms, such as, ethylhexanol, octanol, dodecanol and the like. Examples of aromatic alcohols include benzyl alcohol and the like.

50 In embodiments, the coalescence agent (or coalescing agent or coalescence aid agent) evaporates during later stages of the emulsion/aggregation process, such as, during a second heating step, that is, generally above the  $T_g$  of the resin or a polymer. The final toner particles are thus, free of, or essentially or substantially free of any remaining coalescence agent. To the extent that any remaining coalescence agent may be present in a final toner particle, the amount of remain-

ing coalescence agent is such that presence thereof does not affect any properties or the performance of the toner or developer.

The coalescence agent can be added prior to the coalescence or fusing step in any desired or suitable amount. For example, the coalescence agent can be added in an amount of from about 0.01 to about 10% by weight, based on the solids content in the reaction medium, or from about 0.05, or from about 0.1%, to about 0.5 or to about 3.0% by weight, based on the solids content in the reaction medium. Of course, amounts outside those ranges can be used, as desired.

In embodiments, the coalescence agent can be added at any time between aggregation and coalescence, although in some embodiments it may be desirable to add the coalescence agent after aggregation is, "frozen," or completed, for example, by adjustment of pH, for example, by addition, for example, of base.

Coalescence may proceed and be accomplished over a period of from about 0.1 to about 9 hours, in embodiments, from about 0.5 to about 4 hours.

After coalescence, the mixture may be cooled to room temperature, such as, from about 20° C. to about 25° C. The cooling may be rapid or slow, as desired. A suitable cooling method may include introducing cold water in a jacket around the reactor. After cooling, the toner particles optionally may be washed with water and then dried. Drying may be accomplished by any suitable method for drying including, for example, freeze drying.

#### d. Shells

In embodiments, an optional shell may be applied to the formed toner particles, aggregates or coalesced particles. Any polymer, including those described above as suitable for the core, may be used for the shell. The shell polymer may be applied to the particles or aggregates by any method within the purview of those skilled in the art.

In embodiments, an amorphous polyester resin may be used to form a shell over the particles or aggregates to form toner particles or aggregates having a core-shell configuration. In some embodiments, a low molecular weight amorphous polyester resin may be used to form a shell over the particles or aggregates.

In embodiments, the shell can comprise one or more colorants.

The shell polymer may be present in an amount of from about 10% to about 32% by weight of the toner particles or aggregates, in embodiments, from about 24% to about 30% by weight of the toner particles or aggregates.

Once the desired final size of the toner particles or aggregates is achieved, the pH of the mixture may be adjusted with base to a value of from about 6 to about 10, in embodiments, from about 6.2 to about 7. The adjustment of pH may be used to freeze, that is, to stop, toner particle growth. The base used to stop toner particle growth may be, for example, an alkali metal hydroxide, such as, for example, sodium hydroxide, potassium hydroxide, ammonium hydroxide, combinations thereof and the like. In embodiments, EDTA may be added to assist adjusting the pH to the desired value.

The base may be added in amounts from about 2 to about 25% by weight of the mixture, in embodiments, from about 4 to about 10% by weight of the mixture. Following aggregation to the desired particle size, with the formation of an optional shell as described above, the particles then may be coalesced to the desired final shape, the coalescence being achieved by, for example, heating the mixture to a temperature of from about 55° C. to about 100° C., in embodiments, from about 65° C. to about 75° C., in embodiments, about 70° C., which may be below the melting point of the resin or

polymer(s) to prevent plasticization. Higher or lower temperatures may be used, it being understood that the temperature is a function of the polymer(s) used for the core and/or shell.

#### e. Optional Additives

In embodiments, the toner particles also may contain other optional additives.

##### i. Charge Additives

The toner may include any known charge additives in amounts of from about 0.1 to about 10 weight %, in embodiments, of from about 0.5 to about 7 weight % of the toner. Examples of such charge additives include alkyl pyridinium halides, bisulfates, the charge control additives of U.S. Pat. Nos. 3,944,493; 4,007,293; 4,079,014; 4,394,430; and 4,560,635, the disclosures of each of which are hereby incorporated by reference in entirety, negative charge enhancing additives, such as, aluminum complexes, and the like.

Charge enhancing molecules can be used to impart either a positive or a negative charge on a toner particle. Examples

20 include quaternary ammonium compounds, see, for example, U.S. Pat. No. 4,298,672, organic sulfate and sulfonate compounds, see for example, U.S. Pat. No. 4,338,390, cetyl pyridinium tetrafluoroborates, distearyl dimethyl ammonium methyl sulfate, aluminum salts and so on.

25 Such enhancing molecules can be present in an amount of from about 0.1 to about 10% or from about 1 to about 3% by weight.

##### ii. Surface Modifications

Surface additives can be added to the toner compositions of 30 the present disclosure, for example, after washing or drying. Examples of such surface additives include, for example, one or more of a metal salt, a metal salt of a fatty acid, a colloidal silica, a metal oxide, such as, TiO<sub>2</sub> (for example, for improved RH stability, tribo control and improved development and 35 transfer stability), an aluminum oxide, a cerium oxide, a strontium titanate, SiO<sub>2</sub>, mixtures thereof and the like. Examples of such additives include those disclosed in U.S. Pat. Nos. 3,590,000; 3,720,617; 3,655,374; and 3,983,045, the disclosures of each of which are hereby incorporated by 40 reference in entirety.

Surface additives may be used in an amount of from about 0.1 to about 10 wt %, or from about 0.5 to about 7 wt % of the toner.

Other surface additives include lubricants, such as, a metal 45 salt of a fatty acid (e.g., zinc or calcium stearate) or long chain alcohols, such as, UNILIN 700 available from Baker Petrolite and AEROSIL R972® available from Degussa. The coated silicas of U.S. Pat. Nos. 6,190,815 and 6,004,714, the disclosures of each of which hereby are incorporated by reference in 50 entirety, also can be present. The additive can be present in an amount of from about 0.05 to about 5%, and in embodiments, of from about 0.1 to about 2% of the toner, which additives can be added during the aggregation or blended into the formed toner product.

55 Silica, for example, can enhance toner flow, tribo control, admix control, improved development and transfer stability and higher toner blocking temperature. Zinc, calcium or magnesium stearate also can provide developer conductivity, tribo enhancement, higher toner charge and charge stability. The external surface additives can be used with or without a coating or shell.

The gloss of a toner may be influenced by the amount of 60 retained metal ion, such as, Al<sup>3+</sup>, in a particle. The amount of retained metal ion may be adjusted further by the addition of a chelator, such as, EDTA. In embodiments, the amount of retained catalyst, for example, Al<sup>3+</sup>, in toner particles of the present disclosure may be from about 0.1 pph to about 1 pph,

in embodiments, from about 0.25 pph to about 0.8 pph, in embodiments, about 0.5 pph. The gloss level of a toner of the instant disclosure may have a gloss, as measured by Gardner gloss units (ggu), of from about 20 ggu to about 100 ggu, in embodiments, from about 50 ggu to about 95 ggu, in embodiments, from about 60 ggu to about 90 ggu.

Hence, a particle can contain at the surface one or more silicas, one or more metal oxides, such as, a titanium oxide and a cerium oxide, a lubricant, such as, a zinc stearate and so on. In some embodiments, a particle surface can comprise two silicas, two metal oxides, such as, titanium oxide and cerium oxide, and a lubricant, such as, a zinc stearate. All of those surface components can comprise about 5% by weight of a toner particle weight. There can also be blended with the toner compositions, external additive particles including flow aid additives, which additives may be present on the surface of the toner particles. Examples of these additives include metal oxides like titanium oxide, tin oxide, mixtures thereof, and the like; colloidal silicas, such as AEROSIL®, metal salts and metal salts of fatty acids, including zinc stearate, aluminum oxides, cerium oxides, and mixtures thereof. Each of the external additives may be present in embodiments in amounts of from about 0.1 to about 5 wt %, or from about 0.1 to about 1 wt %, of the toner. Several of the aforementioned additives are illustrated in U.S. Pat. Nos. 3,590,000, 3,800,588, and 6,214,507, the disclosures which are incorporated herein by reference.

Toners may possess suitable charge characteristics when exposed to extreme relative humidity (RH) conditions. The low humidity zone (C zone) may be about 10° C. and 15% RH, while the high humidity zone (A zone) may be about 28° C. and 85% RH.

Toners of the instant disclosure also may possess a parent toner charge per mass ratio (q/m) of from about -5  $\mu$ C/g to about -90  $\mu$ C/g, and a final toner charge after surface additive blending of from about -15  $\mu$ C/g to about -80  $\mu$ C/g.

Other desirable characteristics of a toner include storage stability, particle size integrity, high rate of fusing to the substrate or receiving member, sufficient release of the image from the photoreceptor, nondocument offset, use of smaller-sized particles and so on, and such characteristics can be obtained by including suitable reagents, suitable additives or both, and/or preparing the toner with particular protocols.

The dry toner particles, exclusive of external surface additives, may have the following characteristics: (1) volume average diameter (also referred to as "volume average particle diameter") of from about 2.5 to about 20  $\mu$ m, from about 2.75 to about 10  $\mu$ m, in embodiments, from about 3 to about 7.5  $\mu$ m, from about 5 to about 6  $\mu$ m; (2) number average geometric standard deviation ( $GSD_n$ ) and/or volume average geometric standard deviation ( $GSD_v$ ) of from about 1.17 to about 1.30, from about 1.18 to about 1.28, in embodiments, from about 1.21 to about 1.24; and (3) circularity of from about 0.9 to about 1.0 (measured with, for example, a Sysmex FPIA 2100 analyzer), in embodiments, from about 0.95 to about 0.985, in embodiments, from about 0.96 to about 0.98, from about 0.965 to about 0.97.

### III. Developers

#### A. Composition

The toner particles thus formed may be formulated into a developer composition. For example, the toner particles may be mixed with carrier particles to achieve a two component developer composition. The toner concentration in the developer may be from about 1% to about 25% by weight of the total weight of the developer, in embodiments, from about 2% to about 15% by weight of the total weight of the developer, with the remainder of the developer composition being the

carrier. However, different toner and carrier percentages may be used to achieve a developer composition with desired characteristics.

##### 1. Carrier

Examples of carrier particles for mixing with the toner particles include those particles that are capable of triboelectrically obtaining a charge of polarity opposite to that of the toner particles. Illustrative examples of suitable carrier particles include granular zircon, granular silicon, glass, steel, nickel, ferrites, iron ferrites, silicon dioxide, one or more polymers and the like. Other carriers include those disclosed in U.S. Pat. Nos. 3,847,604; 4,937,166; and 4,935,326.

In embodiments, the carrier particles may include a core with a coating thereover, which may be formed from a polymer or a mixture of polymers that are not in close proximity thereto in the triboelectric series, such as, those as taught herein or as known in the art. The coating may include fluoropolymers, such as polyvinylidene fluorides, terpolymers of styrene, methyl methacrylates, silanes, such as triethoxy silanes, tetrafluoroethylenes, other known coatings and the like. For example, coatings containing polyvinylidene fluoride, available, for example, as KYNAR 301 F™, and/or polymethylmethacrylate (PMMA), for example, having a weight average molecular weight of about 300,000 to about 350,000, such as, commercially available from Soken, may be used. In embodiments, PMMA and polyvinylidene fluoride may be mixed in proportions of from about 30 to about 70 wt % to about 70 to about 30 wt %, in embodiments, from about 40 to about 60 wt % to about 60 to about 40 wt %. The coating may have a coating weight of, for example, from about 0.1 to about 5% by weight of the carrier, in embodiments, from about 0.5 to about 2% by weight of the carrier.

In embodiments, PMMA, for example, may be copolymerized with any desired monomer, so long as the resulting copolymer retains a suitable particle size. Suitable monomers include monoalkyl or dialkyl amines, such as, a dimethylaminoethyl methacrylate, diethylaminoethyl methacrylate, diisopropylaminoethyl methacrylate or butylaminoethyl methacrylate, and the like.

Various effective suitable means can be used to apply the polymer to the surface of the carrier core, for example, cascade roll mixing, tumbling, milling, shaking, electrostatic powder cloud spraying, fluidized bed mixing, electrostatic disc processing, electrostatic curtain processing, combinations thereof and the like. The mixture of carrier core particles and polymer then may be heated to enable the polymer to melt and to fuse to the carrier core. The coated carrier particles then may be cooled and thereafter classified to a desired particle size.

The carrier particles may be prepared by mixing the carrier core with polymer in an amount from about 0.05 to about 10% by weight, in embodiments, from about 0.01 to about 3% by weight, based on the weight of the coated carrier particle, until adherence thereof to the carrier core is obtained, for example, by mechanical impaction and/or electrostatic attraction.

In embodiments, suitable carriers may include a steel core, for example, of from about 25 to about 100  $\mu$ m in size, in embodiments, from about 50 to about 75  $\mu$ m in size, coated with about 0.5% to about 10% by weight, in embodiments, from about 0.7% to about 5% by weight of a polymer mixture including, for example, methylacrylate and carbon black, using the process described, for example, in U.S. Pat. Nos. 5,236,629 and 5,330,874.

#### IV. Devices Comprising a Toner Particle

Toners and developers can be combined with a number of devices ranging from enclosures or vessels, such as, a vial, a

bottle, a flexible container, such as a bag or a package, and so on, to devices that serve more than a storage function.

#### A. Imaging Device Components

The toner compositions and developers of interest can be incorporated into devices dedicated, for example, to delivering same for a purpose, such as, forming an image. Hence, particularized toner delivery devices are known, see, for example, U.S. Pat. No. 7,822,370, and can contain a toner preparation or developer of interest. Such devices include cartridges, tanks, reservoirs and the like, and can be replaceable, disposable or reusable. Such a device can comprise a storage portion; a dispensing or delivery portion; and so on; along with various ports or openings to enable toner or developer addition to and removal from the device; an optional portion for monitoring amount of toner or developer in the device; formed or shaped portions to enable siting and seating of the device in, for example, an imaging device; and so on.

#### B. Toner or Developer Delivery Device

A toner or developer of interest may be included in a device dedicated to delivery thereof, for example, for recharging or refilling toner or developer in an imaging device component, such as, a cartridge, in need of toner or developer, see, for example, U.S. Pat. No. 7,817,944, wherein the imaging device component may be replaceable or reusable.

#### V. Imaging Devices

The toners or developers can be used for electrostaticographic or electrophotographic processes, including those disclosed in U.S. Pat. No. 4,295,990, the disclosure of which hereby is incorporated by reference in entirety. In embodiments, any known type of image development system may be used in an image developing device, including, for example, magnetic brush development, jumping single component development, hybrid scavengerless development (HSD) and the like. Those and similar development systems are within the purview of those skilled in the art.

Imaging processes include, for example, preparing an image with an electrophotographic device including, for example, one or more of a charging component, an imaging component, a photoconductive component, a developing component, a transfer component, a fusing component and so on. The electrophotographic device may include a high speed printer, a color printer and the like.

Once the image is formed with toners/developers via a suitable image development method, such as any of the aforementioned methods, the image then may be transferred to an image receiving medium or substrate, such as, a paper and the like. In embodiments, the fusing member or component, which can be of any desired or suitable configuration, such as, a drum or roller, a belt or web, a flat surface or platen, or the like, may be used to set the toner image on the substrate. Optionally, a layer of a liquid, such as, a fuser oil can be applied to the fuser member prior to fusing.

Color printers commonly use four housings carrying different colors to generate full color images based on black plus the standard printing colors, cyan, magenta and yellow. However, in embodiments, additional housings may be desirable, including image generating devices possessing five housings, six housings or more, thereby providing the ability to carry additional toner colors to print an extended range of colors (extended gamut).

The following Examples illustrate embodiments of the instant disclosure. The Examples are intended to be illustrative only and are not intended to limit the scope of the present disclosure. Parts and percentages are by weight unless other-

wise indicated. As used herein, "room temperature," (RT) refers to a temperature of from about 20° C. to about 30° C.

#### EXAMPLES

5

##### Comparative Control Example

To a 2 liter buchi reactor equipped with an overhead mixer were added 97.19 g of polyester A ( $M_w=86,000$ ,  $T_g$  onset=56° C., 36.9 wt %), 101.42 g of polyester B ( $M_w=19,400$ ,  $T_g$  onset=60° C., 35.43 wt %), 34.06 g crystalline polyester C ( $M_w=23,300$ ,  $M_n=10,500$ ,  $T_m=71$ ° C., 34.98 wt %), 50.64 g polymethylene wax emulsion ( $T_m=90$ ° C., 31.88 wt %), The International Group, Inc. (IGI)), 96.01 g carbon black dispersion (NIPex 35®, 17.00 wt %, Evonik) and 18.27 g cyan pigment PB15:3 (17.00 wt %). After adjusting the pH of the toner reaction slurry to 3.2 using 0.3M  $HNO_3$  solution, 87.45 g  $Al_2(SO_4)_3$  (1 wt %) were added in as a flocculent under homogenization. The mixture was heated to 41.9° C. for aggregation at 460 rpm. The particle size was monitored with a Coulter Counter until the core particles reached a volume average particle size of 4.83  $\mu m$  with a GSD volume of 1.21. Then a mixture of 82.32 g and 85.82 g of the above mentioned polyester resin A and polyester resin B emulsions, respectively, were added to form a shell, resulting in core-shell particles with an average particle size of about 5.48  $\mu m$  and GSD volume of 1.17. Thereafter, the pH of the reaction slurry was increased to 7.87 using 4 wt % NaOH and 6.73 g Versene 100 EDTA (39%) were added to freeze toner growth. After freezing, the reaction mixture was heated to 86.5° C. and the pH was reduced to 6.50 at 85° C. for coalescence. The toner was quenched after coalescence and had a final particle size of about 5.48  $\mu m$  a GSD volume of 1.19 and circularity of about 0.977. The toner slurry was then cooled to room temperature, separated by sieving (25  $\mu m$ ) and filtration, followed by washing and then freeze-drying. In the control toner, all of the pigment was incorporated into the beginning mixture of resin reagents.

40

##### Experimental Example

To a 2 liter glass reactor equipped with an overhead mixer were added 62.57 g of polyester A (38.5 wt %), 66.41 g of polyester B (37 wt %), 23.04 g crystalline polyester C (35.6 wt %), 36.45 g polymethylene wax emulsion (30.37 wt %), 20.91 g carbon black dispersion (NIPex 35®, 16.61 wt %) and 3.42 g cyan pigment PB15:3 (17.21 wt %). After adjusting the pH of the toner reaction slurry to 3.2 using 0.3M  $HNO_3$  solution, 59.84 g  $Al_2(SO_4)_3$  (1 wt %) were added under homogenization. When the toner particles attained an average size of 2.72  $\mu m$ , then 46.47 g more NIPex 35® dispersion and 7.60 g more PB15:3 dispersion were added to the above mixture under homogenization. The mixture was heated to 41.9° C. for aggregation at 250 rpm. The particle size was monitored with a Coulter Counter until the core particles reached a volume average particle size of 5.20  $\mu m$  with a GSD volume of 1.21. Then a mixture of 56.24 g and 52.99 g of the above mentioned polyester resin B and polyester resin A emulsions, respectively, were added to form a shell, resulting in core-shell particles with an average particle size of about 6.08  $\mu m$  and GSD volume of 1.18. Thereafter, the pH of the reaction slurry was increased to 8.5 using 4 wt % NaOH and 4.62 g Versene 100 EDTA (39%) was added to freeze toner growth. After freezing, the reaction mixture was heated to 85° C. and the pH was reduced to 6.08 at 85° C. for coalescence. The toner was quenched after coalescence and had a final particle size of about 6.10  $\mu m$  a GSD volume of 1.21 and

circularity of about 0.965. The toner slurry was then cooled to room temperature, separated by sieving (25  $\mu\text{m}$ ) and filtration, followed by washing and then freeze-drying. In the control toner, all of the pigments were incorporated into the beginning mixture of resin reagents.

#### Results

The resulting particles of both preparations had a narrow particle size distribution.

Due to high conductivity of carbon black pigment, previous hyperpigmented black toners have low charging with high dielectric loss, both of which reduce transfer efficiency and degrade image quality. Amorphous latex can be added to a toner shell to encapsulate the pigment containing core to prevent the pigment as well as other conductive materials, such as, a paraffin wax, from reaching the surface of the toner particle and decreasing toner charge. However, in hyperpigmented toners, black toners and so on, where the colorants may be very conductive or where colorant loading is increased by, for example, up to 45% to enable low TMA, even increasing shell loading may not necessarily ensure good charging.

By adding carbon black dispersion in two portions during the toner aggregation process (i.e., where part of the pigment addition is delayed to after the introduction of the aggregating factor, the toner particles have aggregated to about, for example, about 2 to about 3  $\mu\text{m}$ ), it can be seen in the Table below that the resulting experimental toner particles, which were structurally the same as the control toner particles as to size and circularity, for example, have improved A zone charging.

Further, while not being bound by theory, by sectioning the addition of pigment, it is believed pigment is better distributed in the toner core, which reduced contact of pigment particles, and therefore, reduced formation of conductive pathways when black colorants are used and thereby enhancing charging of toner particles.

Moreover, after the shell layer free of pigment was added, toner charging also was improved.

| Particle             | A zone | C zone | RH sensitivity |
|----------------------|--------|--------|----------------|
| Control example      | -3.4   | -9.9   | 2.91           |
| Experimental example | -4.2   | -9.7   | 2.31           |

It will be appreciated that various of the above-disclosed and other features and functions, or alternatives thereof, may be desirably combined into many other different systems or applications. Also, various presently unforeseen or unanticipated alternatives, modifications, variations or improvements therein may be subsequently made by those skilled in the art, which are also intended to be encompassed by the following claims. Unless specifically recited in a claim, steps or components of claims should not be implied or imported from the specification or any other claims as to any particular order, number, position, size, shape, angle, color or material.

All references cited herein are herein incorporated by reference in entirety.

We claim:

1. A method for making a toner particle comprising the following steps:

a. combining an amorphous resin, an optional crystalline resin, a first colorant and an optional wax to form an emulsion;

b. mixing said emulsion to form particles;

c. adding an aggregating factor to said emulsion; and

d. aggregating said particles to form toner particles,

wherein a second colorant is added in portions in one or more of said steps, wherein the first and second colorants may be the same or different.

2. The method of claim 1, further comprising coalescing said toner particles.

3. The method of claim 1, further comprising adding a shell to said toner particles.

4. The method of claim 1, further comprising adding surface additives to said toner particles.

5. The method of claim 1, further comprising combining said toner particles with a carrier to form a developer.

6. The method of claim 5, wherein said developer comprising said toner particles has A zone charging which is improved as compared to that of a developer comprising toner particles prepared by adding colorant to said composition prior to said mixing step.

7. The method of claim 1, wherein said amorphous resin comprises a low molecular weight amorphous resin, a high molecular weight amorphous resin or both.

8. The method of claim 1, wherein said toner particle is hyperpigmented.

9. The method of claim 1, wherein the first or second colorant comprises a colored pigment other than a black pigment.

10. The method of claim 1, wherein said first or second colorant comprises a black colorant.

11. The method of claim 10, wherein said black colorant comprises one or more of the following properties: a BET surface area of about 65  $\text{m}^2/\text{g}$ ; an OAN of about 42 ml/100 g or about 0.5% volatile matter at 950° C.

12. The method of claim 1, further comprising an additional colorant.

13. The method of claim 12, wherein said additional colorant is added in portions or continuously in one or more of said steps.

14. The method of claim 12, wherein said additional colorant comprises a cyan colorant.

15. The method of claim 12, wherein the ratio of the first colorant to the additional colorant is in a weight ratio of from 20:1 to 1:1.

16. The method of claim 1, wherein said first colorant is added in two portions, the amount of the first portion of the first colorant and the second portion of the first colorant as a ratio by weight is from 1:9 to 9:1.

17. The method of claim 1, wherein the toner particles comprise from about 4% to about 45% colorants.

18. The method of claim 1, wherein said toner particle is from about 5 to about 6  $\mu\text{m}$  in diameter.

19. The method of claim 1, wherein said toner particle has a circularity of from about 0.95 to about 0.985.

20. The method of claim 1, wherein said toner particle has a GSD volume of from about 1.17 to about 1.30.